

July 22, 1958

2,844,492

E. FITZER  
METHOD OF PRODUCING HEAT RESISTING METALLIC  
MATERIALS AND FORMED BODIES  
Filed Feb. 23, 1954

FIG. 1.



INITIAL METAL POWDER



FIG. 2.

CONVERTED METAL  
POWDER AND Mo

FIG. 3.



MOLDING

FIG. 4.

SINTERING

ACTIVATED  
ATMOSPHERE

METALLIC SKELETON  
& METALLIC POWDER

FIG. 5.

SINTERING

ACTIVATED  
ATMOSPHERE

INVENTOR.

ERICH FITZER

BY



ATT'Y.

1

2,844,492

**METHOD OF PRODUCING HEAT RESISTING METALLIC MATERIALS AND FORMED BODIES**

Erich Fitzer, Vienna, Austria, assignor to Siemens-Plania-Werke Aktiengesellschaft fuer Kohlefabrikate, Meitingen, near Augsburg, Germany, a corporation of Germany

Application February 23, 1954, Serial No. 411,949

Claims priority, application Austria February 26, 1953

4 Claims. (Cl. 117—66)

This invention relates to the production of metallic materials and is particularly concerned with a method of producing heat resisting metallic materials, that is, metallic materials which remain substantially constant in the presence of high temperatures and which are adapted for making electrical heating resistors or structural apparatus and machine elements exposed to temperatures on the order of about 1750° C., for example, protective tubing, nozzles, burner heads, parts of gas turbines and the like.

Such materials are made of chemical compositions of the so-called transition metals of the fourth to sixth groups of the periodic system of elements (Ti, Zr, Hf, V, Nb, Ta, Cr, Mo, W) containing semimetals such as Si, B. Disilicides and diborides of molybdenum and chromium are particularly suitable for the above mentioned purposes.

These compositions are also referred to as hard materials because of the great hardness exhibited thereby. Formed or molded bodies are usually produced from these hard materials by powdered metal, taking corresponding initial materials or starting with formed metallic bodies whose metal is converted into the desired semimetal composition.

Of the known methods of producing metallic disilicides and metallic diborides, that method which is of especial technological interest is the one in which the conversion of the metals or their alloys which are to form the hard materials is accomplished with vaporized halogen compounds of boron or silicon. This "vaporizing method" which is applicable for siliconizing or boronizing of metallic powders as well as of metallic bodies has, however, the drawback of requiring long reaction times and exhibiting a spatially differentiated reaction, causing formation of disturbing coatings on the treated metallic bodies.

The invention accelerates the reaction and improves its efficiency, making it not only possible to convert metallic powder or thin bodies of metals forming the hard material into disilicides or diborides but also to form on the surfaces of relatively thick metallic parts a well adhering protective coating of metallic disilicide or metallic diboride, respectively. The volatile halogen compounds offer in addition purification possibilities and therefore the making of purest hard materials free of foreign metallic admixtures.

In accordance with the invention, these advantages are obtained by activating vaporized halides of silicon or boron, prior to the reaction with the metal that is to form the hard material, by conducting it over large surfaces of metallic silicon or boron, at a temperature which causes the formation of unstable halogen compounds. The silicon- or boron-halides are thereby suitably intermixed with a neutral or a reducing carrier gas and are in a heating zone activated by the silicon or boron or alloys thereof.

It was found that the best activation takes place at the highest temperatures provided that the activated

2

chlorides are not subjected to any cooling prior to the vaporization reaction, at any rate, no cooling below the temperature of the vaporization reaction. The activation presumably causes formation of low grade halogen compounds which are unstable at a lower temperature. The catalytic reduction of the semimetal chlorides by the hydrogen carrier gas, during the vaporization reduction or rather the heterogeneous metallic exchange reaction of the semimetal chlorides with the solid metal that is to form the hard material would thus seem to be facilitated and in some cases actually effected by the formation of unstable halogen compounds. These heterogeneous reactions may also be superimposed upon contact with the metallic surface which is at lower temperature by a thermal decomposition of the subchlorides formed at the higher temperatures.

The activation method according to the invention offers the further advantage of permitting incident to circulation of the vaporization atmosphere, in a closed cycle, during the activation, a regeneration of the halogen or hydrogen halides produced in the vaporization reaction.

The method according to the invention may be practiced in various ways, for example, to produce from corresponding metal powders hard material powder for use as an initial substance for making formed or molded bodies by molding or pressing and sintering.

The metals and alloys which are to form the hard material are for this purpose exposed to the treatment while in powdered form at desired particle size. It is merely necessary to provide the greatest possible exposed surface area and to renew continuously the vaporization atmosphere while maintaining the temperature. A slight uniform agitation of the metallic powder is of advantage. The so-called flowing material bed may be advantageously used for forming such hard materials from corresponding metallic powders. It may be mentioned as an example that it is possible to convert molybdenum powder with an average particle size of  $1\mu$ , at 1200° C. in a few minutes completely into  $\text{MoSi}_2$  by the use of silicon chlorides free of HCl and activated at 1300° C. over silicon powder. The resulting disilicide powder can be directly pressed and worked without any prior comminution or screening.

It is possible to produce in this manner heating conductors, structural furnace parts, protective tubing, nozzles, burner heads, parts for turbines and internal combustion engines, in short, all constructional parts and elements which are exposed to temperatures on the order of about 1750° C. Particularly favorable is the constancy of or resistance against  $\text{V}_2\text{O}_5$  corrosion, of such  $\text{MoSi}_2$  bodies made in accordance with the invention, making them usable in internal combustion engines operated with crude oil without having to fear accelerated oxidation by clinkering.

However, these hard metallic disilicides and diborides, for example,  $\text{MoSi}_2$ , can be molded only by the use of very high pressures and their sinterability is wanting at the temperatures that may be reached in a protective gas. Molybdenum powder is added to improve the molding properties of  $\text{MoSi}_2$  powder. In order to convert the metallic powder contained in the powdered mixture, upon sintering, into the corresponding disilicide or diboride, the invention proposes to sinter the molded body in an atmosphere containing activated boron- or silicon-halide. The sinter atmosphere is thereby continuously conducted through the sinter chamber and is subjected to activation prior to entering the sinter chamber by conducting it over metallic boron or silicon. The treatment of the molded body with boron or silicon halide is suitably continued during the sintering until an excess of a semimetal, that is, silicon or boron is precipitated upon the surface of the molded body.

It was found, for example, with disilicides that a particularly favorable oxidation resistance of the treated molded body is present when such body exhibits a relatively low silicon excess as compared with the stoichiometric composition of the disilicide. Such an excess of semimetal which settles in the pores of the hard material body may also be obtained by thermal decomposition of vapor-formed unstable halogen compounds of the semi-metal during the sintering procedure. For this purpose, advantage may be taken, for example, of compounds which are stable at lower temperatures, for example, silicon iodide, which decomposes thermally on the highly heated molded body in known manner. A halogen compound which is stable at higher temperature and which is formed directly prior to decomposition will also decompose incident to cooling upon contacting the molded body, and will thereby precipitate the desired semimetal thereon. Such a thermal decomposition may also take place in the present method when the activation temperature of the vaporlike halogen compound of the semimetal is above the reaction temperature of the metal which is to form the hard material. The catalytic reaction during the vaporizing procedure, that is, the metal exchange reaction between metal and semimetal, for example, molybdenum and silicon, is facilitated by the formation of unstable compounds and is supported by a thermal decomposition of the halogen compositions.

Alloys may also be used for the powdered mixture of the hard materials which is to be sintered, that is, disilicides or diborides of the metals which are to form the hard material. The thermal decomposition of the vaporlike halogen compounds not only causes a conversion of the metallic particles of the sinter body to form the corresponding metallic disilicides or diborides, but there also occurs an enrichment with metallic silicon or boron especially along the surface layer. A sinter body is thus obtained which is characterized by an especially dense surface and which is oxidation proof at high temperatures.

In the treatment of pressed or molded bodies, made of metal powders which are to form hard materials, with activated reaction gas, during the sintering, it is sufficient if this reaction treatment is carried on only during part of the sintering time.

The new method of producing hard materials by conversion of activated halogen compounds of the semimetals with the metals that are to form the hard materials is not limited to the treatment of powders of such materials. It was found that the method is excellently adapted for treating formed or molded bodies made of the corresponding metals. According to the thickness or wall thickness, respectively, of the molded bodies, annealed in a reaction gas, a hard material coating or layer will thereby form upon such bodies or they will undergo conversion into the corresponding hard material. The formation of the hard material layer or coating is accomplished very quickly with the present method, and the layer will accordingly be of fine grain and will not tend to separate. Prior methods provided coarse grained layers or coatings and caused recrystallization of the base metal.

The present method of boronizing or siliconizing transition metals of the fourth to sixth groups of the periodic system may also be advantageously used in cases where highly temperature proof bodies of relatively large dimensions are to be produced which cannot be made solely from powdered metal in molds or press forms. In such cases, the hard material powder is pressed or molded into parts forming a metallic skeleton. The resulting molded body consisting of a powder mixture and a solid metal body is thereafter subjected to sintering in an atmosphere containing activated vaporized halogen

compounds of silicon or boron so that the metallic skeleton part is converted into the corresponding disilicide or diboride at least in its surface layer. The disilicides or diborides which are present penetrate thereby into the metal so that a solid body will result which exhibits great mechanical strength even at high temperatures.

It is possible to produce in this manner, for example, satisfactory heat conductors of  $MoSi_2$  by using molybdenum parts, for example, in the form of concentric tubes and molding  $MoSi_2$  powder into the annular space therebetween. The resulting body is thereafter sintered in an atmosphere containing an activated silicon halogen compound so that the metallic molybdenum tubes are covered with a protective layer of molybdenum disilicide.

It is understood of course that different metallic skeleton bodies may be employed, for example, wires to be used as heaters, and that hard material powder may be molded thereabout to increase the mechanical strength thereof.

It is possible to produce in this manner long thin heater wires with desired resistance, which could not be made before because only relatively short and thick molded bodies could be produced of pressed and sintered pulver mixtures alone which had sufficient mechanical strength.

The various phases of the method described herein are illustrated in identical sequence in the accompanying diagrammatic drawings Fig. 1-5. Known apparatus may be used to carry out the required operations.

What is believed new and desired to have protected by Letters Patent is defined in the appended claims.

I claim:

1. Method of producing high-melting material from a base metal taken from transition metals of the fourth to sixth groups of the periodic system of elements by reaction at elevated temperature of one of said metals with a vaporized halide compound of a semi-metal taken from the group consisting of silicon and boron, comprising forming a vaporized halide of said semi-metal, activating said halide prior to reaction with the base metal by large area contact at elevated temperature with a corresponding metallic semi-metal to form an unstable halide compound, and thereafter causing reaction of said activated halide compound with said base metal, the temperature incident to activation of said halide compound exceeding the temperature required for reaction with said base metal.

2. A method according to claim 1, wherein said base metal is in powdered form.

3. A method according to claim 2, wherein said halide compound is silicon chloride free of  $HCl$  and activated at  $1300^{\circ} C.$  in contact with silicon powder, said base metal being molybdenum powder with an average particle size of  $1\mu$ , reaction of said molybdenum powder with said activated halide compound being effected at  $1200^{\circ} C.$ , said reaction causing conversion of said molybdenum powder to form molybdenum disilicide.

4. A method according to claim 3, comprising molding said molybdenum disilicide to form a desired body, sintering said body, and exposing said body during the sintering thereof to the action of a gas mixture comprising said activated halide and a carrier gas.

#### References Cited in the file of this patent

#### UNITED STATES PATENTS

|    |           |              |               |
|----|-----------|--------------|---------------|
| 65 | 2,206,395 | Gertler      | July 2, 1940  |
|    | 2,307,005 | Ruben        | Dec. 29, 1942 |
|    | 2,657,128 | Stern et al. | Oct. 27, 1953 |

#### FOREIGN PATENTS

|    |         |               |                |
|----|---------|---------------|----------------|
| 70 | 435,754 | Great Britain | Sept. 23, 1935 |
|    | 598,181 | Great Britain | Feb. 12, 1948  |